



## 3

perfluorodetergent. The blades are sprayed with an aqueous emulsion of a PPFP solution in a perfluoroalkane or, after having been previously dried, they may be dipped into the pure solution or its emulsion. Alternatively the pure solution or its emulsion may be sprayed on the blades. The blades are then dried and preferably heated for five minutes to several hours at temperatures exceeding 190° C. In the case of carbon steel blades it is best to keep the temperature under 250° C. A protective gas atmosphere is unnecessary until the temperatures exceed 250° C. if such high temperatures are to be used. Otherwise the blades are simply heated in air. The safety razor blades thus obtained give a shave that is decidedly smooth and this remains so for a large number of shaves.

The invention is illustrated by the following examples.

## EXAMPLE 1

(A) An 0.5% solution of PPFP in perfluoro-1,3-dimethylcyclobutane is emulsified with the aid of an Ultraturrax (mechanical high frequency apparatus for dispersing, dissolving, homogenising and emulsifying for the performance of physical and chemical material changes) in twice the quantity of water containing a perfluorinated emulsifier, such as perfluorocaprylic acid or its ammonium salt, in a dilution of 0.01%. This produces a sprayable emulsion.

(B) A batch of carbon steel razor blades and "ice hardened" chrome steel razor blades was degreased with benzene in a Soxhlet apparatus for two days. After being dried, the cutting edge side of this batch was sprayed with the suspension prepared as set out in Example 1A, from a spray gun. The blades were then dried. The carbon steel blades were heated for one hour at 210° C., whereas the chrome steel blades were heated at 260° C. for fifteen minutes.

## EXAMPLE 2

A batch of blades was degreased as described in Example 1B and sprayed with a solution of PPFP in perfluoroctane. Stoving was as described in Example 1B.

## EXAMPLE 3

A dried chrome steel blade which had been sprayed as described in Examples 1B or 2 was tempered in a protective gas atmosphere at 350° C. for ten minutes.

## 4

## EXAMPLE 4

Blades that had been degreased in the manner described in Example 1B were washed with an aqueous 0.05% solution of ammonium salt of perfluorocarbylic acid and dried. The blades were then further treated in the same way as in Examples 1B, 2 or 3.

The finished coated blades of the above examples had an excellent keenness and gave a very smooth shave for a relatively large number of shaves.

I claim:

1. The process for improving the shaving properties of carbon steel razor blades wherein the cutting edge or edges of mechanically completed and cleaned blades are coated with a solution of polyperfluoropropylene and then heated at a temperature between about 190° C. to 250° C.
2. The process of claim 1 in which said solution is applied to said blade as an emulsion.
3. The method of claim 2 in which said emulsion includes a perfluorinated emulsifier.
4. The method of claim 1 wherein said blade is heated in an atmosphere of air.
5. The method of claim 1 wherein said blade is heated for five minutes to several hours.
6. The method of claim 1 wherein said solution of said polyperfluoropropylene comprises a perfluoroalkane as a solvent for said perfluoropropylene.
7. The method of claim 1 wherein said solution of polyperfluoropropylene is sprayed on to said blade as a suspension.
8. A razor blade made by the method of claim 1.

## References Cited

## UNITED STATES PATENTS

|           |         |              |       |           |
|-----------|---------|--------------|-------|-----------|
| 3,958,685 | 11/1960 | Eleuterio    | ----- | 260—92.1  |
| 3,071,856 | 1/1963  | Fischbein    | ----- | 117—161 X |
| 3,203,829 | 8/1965  | Seyer et al. | ----- | 117—132   |
| 3,206,344 | 9/1965  | Elkins       | ----- | 156—86 X  |
| 3,341,348 | 9/1967  | Letendre     | ----- | 117—8     |
| 3,376,183 | 4/1968  | Flynn et al. | ----- | 156—244   |

RALPH J. KENDALL, Primary Examiner

U.S. Cl. X.R.

30—346.5, 346.53; 117—161